



US008765334B2

(12) **United States Patent**  
**Lin et al.**

(10) **Patent No.:** **US 8,765,334 B2**  
(b5) **Date of Patent:** **Jul. 1, 2014**

(54) **PROTECTIVE PHOTORECEPTOR OUTER LAYER**

(75) Inventors: **Liang-bih Lin**, Rochester, NY (US); **Kenny-Tuan T. Dinh**, Webster, NY (US); **Emily K. Redman**, Webster, NY (US); **Brian P. Gilmartin**, Williamsville, NY (US)

(73) Assignee: **Xerox Corporation**, Norwalk, CT (US)

(\*) Notice: Subject to any disclaimer, the term of this patent is extended or adjusted under 35 U.S.C. 154(b) by 458 days.

(21) Appl. No.: **12/693,354**

(22) Filed: **Jan. 25, 2010**

(65) **Prior Publication Data**

US 2011/0183241 A1 Jul. 28, 2011

(51) **Int. Cl.**  
**G03G 15/00** (2006.01)

(52) **U.S. Cl.**  
USPC ..... **430/56**; 430/60; 430/64; 430/72;  
430/58.05

(58) **Field of Classification Search**

USPC ..... 430/60, 64, 66, 72, 125, 58.05  
See application file for complete search history.

(56) **References Cited**

U.S. PATENT DOCUMENTS

|               |        |                            |
|---------------|--------|----------------------------|
| 3,121,006 A   | 2/1964 | Middleton et al.           |
| 3,937,665 A * | 2/1976 | Mammino et al. .... 134/42 |
| 4,286,033 A   | 8/1981 | Neyhart et al.             |
| 4,291,110 A   | 9/1981 | Lee                        |
| 4,338,387 A   | 7/1982 | Hewitt                     |

|                   |         |                              |
|-------------------|---------|------------------------------|
| 4,387,980 A       | 6/1983  | Ueno et al.                  |
| 4,464,450 A       | 8/1984  | Teuscher                     |
| 4,587,189 A       | 5/1986  | Hor et al.                   |
| 4,921,773 A       | 5/1990  | Melnik et al.                |
| 5,069,993 A       | 12/1991 | Robinette et al.             |
| 5,215,839 A       | 6/1993  | Yu                           |
| 5,660,961 A       | 8/1997  | Yu                           |
| 5,756,245 A       | 5/1998  | Esteghamatian et al.         |
| 5,958,638 A       | 9/1999  | Katayama et al.              |
| 6,004,716 A *     | 12/1999 | Kato et al. .... 430/125.31  |
| 6,713,220 B2      | 3/2004  | Graham et al.                |
| 2003/0180655 A1 * | 9/2003  | Fan et al. .... 430/270.1    |
| 2005/0037274 A1 * | 2/2005  | Shida et al. .... 430/60     |
| 2005/0084783 A1 * | 4/2005  | Yau et al. .... 430/66       |
| 2005/0170273 A1 * | 8/2005  | Fuller et al. .... 430/66    |
| 2006/0210908 A1 * | 9/2006  | Umemura et al. .... 430/125  |
| 2006/0222979 A1 * | 10/2006 | Ishida et al. .... 430/72    |
| 2006/0240346 A1 * | 10/2006 | Toda et al. .... 430/64      |
| 2007/0003850 A1 * | 1/2007  | Yamada et al. .... 430/58.05 |
| 2007/0148575 A1 * | 6/2007  | Mishra et al. .... 430/66    |
| 2009/0004588 A1 * | 1/2009  | Sheng et al. .... 430/83     |

\* cited by examiner

*Primary Examiner* — Mark F Huff

*Assistant Examiner* — Rashid Alam

(74) *Attorney, Agent, or Firm* — Pillsbury Winthrop Shaw Pittman LLP

(57) **ABSTRACT**

Embodiments pertain to a novel imaging member, namely, an imaging member or photoreceptor comprising a protective outer layer which comprises light-absorbing composition that substantially prevents any light absorption by the overcoat layer. The composition comprises a low strength thermal plastic resin and a high optical density yellow dye. Thus, the light-blocking protective layer reduces the intrinsic light shock suffered by conventional overcoat layers without negatively impacting electrical properties of the overcoat layer and while improving print quality.

**12 Claims, 4 Drawing Sheets**





FIG. 1



FIG. 2



**FIG. 3**



FIG. 4



FIG. 5

## PROTECTIVE PHOTORECEPTOR OUTER LAYER

## BACKGROUND

The present embodiments pertain to a novel imaging member, namely, an imaging member or photoreceptor comprising a protective outer layer which comprises light-blocking composition that substantially prevents any light absorption by the overcoat layer. The composition comprises a low strength thermal plastic resin and a high optical density yellow dye with a molar extinction coefficient of  $5000\text{ M}^{-1}\text{ cm}^{-1}$  or higher. In this manner, the light-blocking protective layer reduces the intrinsic light shock suffered by conventional overcoat layers without negatively impacting electrical properties of the overcoat layer and while improving print quality.

In electrophotographic or electrophotographic printing, the charge retentive surface, typically known as a photoreceptor, is electrostatically charged, and then exposed to a light pattern of an original image to selectively discharge the surface in accordance therewith. The resulting pattern of charged and discharged areas on the photoreceptor form an electrostatic charge pattern, known as a latent image, conforming to the original image. The latent image is developed by contacting it with a finely divided electrostatically attractive powder known as toner. Toner is held on the image areas by the electrostatic charge on the photoreceptor surface. Thus, a toner image is produced in conformity with a light image of the original being reproduced or printed. The toner image may then be transferred to a substrate or support member (e.g., paper) directly or through the use of an intermediate transfer member, and the image affixed thereto to form a permanent record of the image to be reproduced or printed. Subsequent to development, excess toner left on the charge retentive surface is cleaned from the surface. The process is useful for light lens copying from an original or printing electronically generated or stored originals such as with a raster output scanner (ROS), where a charged surface may be imagewise discharged in a variety of ways.

The described electrophotographic copying process is well known and is commonly used for light lens copying of an original document. Analogous processes also exist in other electrophotographic printing applications such as, for example, digital laser printing or ionographic printing and reproduction where charge is deposited on a charge retentive surface in response to electronically generated or stored images.

To charge the surface of a photoreceptor, a contact type charging device has been used. The contact type charging device includes a conductive member which is supplied a voltage from a power source with a D.C. voltage superimposed with a A.C. voltage of no less than twice the level of the D.C. voltage. The charging device contacts the image bearing member (photoreceptor) surface, which is a member to be charged. The outer surface of the image bearing member is charged with the rubbing friction at the contact area. The contact type charging device charges the image bearing member to a predetermined potential. Typically the contact type charger is in the form of a roll charger such as that disclosed in U.S. Pat. No. 4,387,980, the relative portions thereof incorporated herein by reference.

Multilayered photoreceptors or imaging members have at least two layers, and may include a substrate, a conductive layer, an optional undercoat layer (sometimes referred to as a "charge blocking layer" or "hole blocking layer"), an optional adhesive layer (sometimes referred to as an "interfacial layer"), a photogenerating layer (sometimes referred to as a

"charge generation layer," "charge generating layer," or "charge generator layer"), a charge transport layer, and an optional overcoating layer in either a flexible belt form or a rigid drum configuration. In the multilayer configuration, the active layers of the photoreceptor are the charge generation layer (CGL) and the charge transport layer (CTL). Enhancement of charge transport across these layers provides better photoreceptor performance. Multilayered flexible photoreceptor members may include an anti-curl layer on the backside of the substrate, opposite to the side of the electrically active layers, to render the desired photoreceptor flatness.

The electrical properties of some photoreceptors can change upon exposure to light, and these undesirable changes can result in poor print quality. Past studies have shown that this problem is caused by light shock, which is in turn due to the interaction of blue light with the photogenerating layer. In the case of organic photoreceptors having an overcoat layer, it has been discovered that the light shock is intrinsic to the overcoat layer itself and strongly wavelength dependent (e.g., the majority of the light shock being caused by 400-500 nm light).

In the case of overcoated drum photoreceptors, light shock occurs during replacement of xerographic customer replacement units (CRU) and/or photoreceptor service where the unit is exposed to ambient light for over 1 to 2 minutes. Standard overcoat layers are known to absorb in the ultraviolet (UV) region of 450 nm or less, indicating that the UV component of sun light or fluorescent room light is the major cause of light shock which is manifested as a local change in image density (darkening or lightening) due to a local change in charge transport properties induced by UV or visual light. The typical life time of the defect can be as long as several days.

Prior solutions focused on the interaction of light with the photogenerating layer but did not address intrinsic overcoat layer light shock protection. For example, U.S. Pat. No. 6,713,220, incorporated herein by reference, discloses a method for reducing the effects of light shock by preventing 400-500 nm light from interacting with the generator layer by doping a light-absorbing material into a charge transport layer comprising arylamine. However, intrinsic light shock observed in organic overcoat layers is not resolved by the method taught by U.S. Pat. No. 6,713,220. Thus, there is a need for a solution to the intrinsic light shock experienced by organic overcoat layers.

Conventional photoreceptors are disclosed in the following patents, a number of which describe the presence of light scattering particles in the undercoat layers: Yu, U.S. Pat. No. 5,660,961; Yu, U.S. Pat. No. 5,215,839; and Katayama et al., U.S. Pat. No. 5,958,638. The term "photoreceptor" or "photocconductor" is generally used interchangeably with the terms "imaging member." The term "electrophotographic" includes "electrophotographic" and "xerographic." The terms "charge transport molecule" are generally used interchangeably with the terms "hole transport molecule."

## SUMMARY

According to aspects illustrated herein, there is provided a protective outer film for an imaging member, comprising a low-strength film-forming thermal plastic resin, and a yellow dye, wherein the protective outer film blocks ultraviolet or visible light in the range of from about 400 nm to about 515 nm.

In another embodiment, there is provided a light shock resistant imaging member, comprising a substrate, a charge generation layer disposed on the substrate, a charge transport layer disposed on the charge generation layer, an overcoat

layer disposed on the charge transport layer, and a protective outer film, comprising a low-strength film-forming thermal plastic resin, and a yellow dye, wherein the protective outer film blocks ultraviolet or visible light in the range of from about 400 nm to about 515 nm from the imaging member.

Yet another embodiment, there is provided an image forming apparatus for forming images on a recording medium comprising a) a light shock resistant imaging member having a charge retentive-surface for receiving an electrostatic latent image thereon, wherein the imaging member comprises a substrate, a charge generation layer disposed on the substrate, a charge transport layer disposed on the charge generation layer, an overcoat layer disposed on the charge transport layer, and a protective outer film, comprising a low-strength film-forming thermal plastic resin, and a yellow dye, wherein the protective outer film blocks ultraviolet or visible light in the range of from about 400 nm to about 515 nm from the imaging member, b) a development component for applying a developer material to the charge-retentive surface to develop the electrostatic latent image to form a developed image on the charge-retentive surface, c) a transfer component for transferring the developed image from the charge-retentive surface to a copy substrate, d) a fusing component for fusing the developed image to the copy substrate, and e) cleaning component for removing any developer material remaining on the charge-retentive surface, wherein the cleaning component removes the removable protective layer after a first few cycles of operation of the image forming apparatus and directs the removed developer material to a toner waste container.

#### BRIEF DESCRIPTION OF THE DRAWINGS

For a better understanding, reference may be made to the accompanying figures.

FIG. 1 is a cross-sectional view of an imaging member in a drum configuration according to the present embodiments;

FIG. 2 is a cross-sectional view of an imaging member in a belt configuration according to the present embodiments;

FIG. 3 is a marginal means plot of difference in surface potential at exposure of 1.86 ergs/cm<sup>2</sup> ( $\Delta V_{low}$ ) for factors in charge generation layer thickness (CG pull rate of 130 and 250 mm/minute), extra heating, and overcoat types;

FIG. 4 is an absorption spectra of overcoat and various dyes according to the present embodiments; and

FIG. 5 is the differences in erase voltage (Verase) and  $V_{low}$  at 1.86 ergs/cm<sup>2</sup> of an imaging member having a conventional overcoat layer and an imaging member having the inventive overcoat layer according to the present embodiments.

#### DETAILED DESCRIPTION

In the following description, reference is made to the accompanying drawings, which form a part hereof and which illustrate several embodiments. It is understood that other embodiments may be used and structural and operational changes may be made without departure from the scope of the present disclosure.

The presently disclosed embodiments generally pertain to a novel imaging member or photoreceptor which comprises a protective outer layer that exhibits absorbs UV and/or visible light and thus protects the imaging member from light shock. As compared to the conventional imaging members without the protective layers, the inventive imaging members having the removable protective layer exhibit improved print quality.

Conventional polymeric anti-scratch overcoat (PASCO) photoreceptors have been observed to suffer over 100V

decreases in  $V_{low}$  and  $V_{er}$  after light shock, which is mainly attributed to the thick charge generation layer needed for meeting  $V_{low}$  specification and withstand extra heating during the overcoat curing. In addition, when installing new cartridges, there is the potential of exposing the imaging member to light for up to several minutes. The "light shock" will cause overdevelopment in darker prints and the recovery takes several days to weeks. Thus, light shock becomes a substantial obstacle for long-life imaging members and a main drawback for the total cost of ownership (TCO) reduction. Previous methods of protection focused on modifying the charge transport layer or charge generation layer, but those investigations ended without much success.

The present embodiments help resolve the above-described problems by applying a thin non-acting yellow dye film to form a protective outer layer on top of the PASCO overcoat photoreceptors to prevent light shock. The film is comprised of a low strength thermal plastic resin and a high optical density yellow dye. In the present embodiments, a low strength thermal plastic resin is one that does not crosslink and which is generally identified as a low molecular weight thermal plastic with low mechanical strength that can be easily worn off by any force. The strong absorbing dye blocks off visible light in the wavelength range of from about 400 nm to about 515 nm, the most sensitive region of light known to induce light shock. The protective outer layer can be applied and removed with a non-toxic solvent such as isopropanol. Due to the low strength of the resin, the protective outer layer also does not last for many copies in print engines and thus will be entirely removed after a few cycles—making it a true sacrificial layer for light shock reduction. Therefore, the protective outer layer protects the photoreceptor from light shock during the initial installation of the photoreceptor cartridge and like CRU, and can subsequently be removed with an appropriate solvent or be removed after the initial cycles.

The exemplary embodiments of this disclosure are described below with reference to the drawings. The specific terms are used in the following description for clarity, selected for illustration in the drawings and not to define or limit the scope of the disclosure. The same reference numerals are used to identify the same structure in different figures unless specified otherwise. The structures in the figures are not drawn according to their relative proportions and the drawings should not be interpreted as limiting the disclosure in size, relative size, or location. In addition, though the discussion will address negatively charged systems, the imaging members of the present disclosure may also be used in positively charged systems.

FIG. 1 is an exemplary embodiment of a multilayered electrophotographic imaging member having a drum configuration. As can be seen, the exemplary imaging member includes a rigid support substrate 10, an undercoat layer 14, a charge generation layer 18 and a charge transport layer 20. The rigid substrate may be comprised of a material selected from the group consisting of a metal, metal alloy, aluminum, zirconium, niobium, tantalum, vanadium, hafnium, titanium, nickel, stainless steel, chromium, tungsten, molybdenum, and mixtures thereof. The charge generation layer 18 and the charge transport layer 20 forms an imaging layer described here as two separate layers. In an alternative to what is shown in the figure, the charge generation layer may also be disposed on top of the charge transport layer. It will be appreciated that the functional components of these layers may alternatively be combined into a single layer.

FIG. 2 shows an imaging member having a belt configuration according to the embodiments. As shown, the belt configuration is provided with an anti-curl back coating 1, a

supporting substrate **10**, an electrically conductive ground plane **12**, an undercoat layer **14**, an adhesive layer (also referred to an interfacial layer) **16**, a charge generation layer **18**, and a charge transport layer **20**. An optional overcoat layer **32** and ground strip **19** may also be included. An exemplary photoreceptor having a belt configuration is disclosed in U.S. Pat. No. 5,069,993, which is hereby incorporated by reference. Organic photoreceptors usually comprise a metalized substrate, undercoat layer, charge generation layer (CGL) and charge transport layer (CTL), sequentially. To form a latent image on the surface of photoreceptor, a charged photoreceptor has to be exposed by light, which usually is a laser with wavelength in visible light range. The ideal situation would be one in which the charge generation layer could absorb all the incident photons and no exposure light could penetrate through the CGL. In reality, however, there is always a small amount of light that passes through the CGL and UCL, and is then reflected back through the photoreceptor. This light interference results in a print defect.

#### The Protective Outer Layer

The photoreceptors of the present embodiments employ a protective outer layer or film **36** disposed over the overcoat layer **32**. The photoreceptors of the present embodiments provide a protective outer layer or film **36** that exhibits resistance to light shock and also exhibits good electrical performance as compared to conventional photoreceptors that employ only a PASCO overcoat layer without the protective outer layer **36**.

The substantial prevention of interaction between light and the overcoat layer is based on the fact that the protective outer layer blocks light strongly in the 400 to 515 nm range (e.g., absorbs UV/blue light) and thus blocks the majority of light that would otherwise interact with the overcoat layer to interact with the overcoat layer and cause the light shock effect.

In the present embodiments, the protective outer layer **36** is formed from a low strength thermal plastic resin, such as polyvinylbutyral with weight average molecular weight of less 10,000, and a high optical density yellow dye with an extinction coefficient of 5,000 M<sup>-1</sup> cm<sup>-1</sup> or higher. In specific embodiments, the thermal plastic resin is selected from the group consisting of poly-vinyl butyral, polyester, polycarbonate, polystyrene, melamine formaldehyde resins, polyacrylamide, polyurethane, polysulfonate, polyacrylonitrile, polyethylene glycol, poly(methyl acrylate), poly(methyl methacrylate), or the like, and mixtures thereof. In specific embodiments, the yellow dye is selected from the group consisting of metal-free monoazo compounds, 2-2'-dihydroxy-4-methoxybenzophene, oxybenzone, tartrazine, quinophthalone, pyrazolone, methane, coumarin, and chromium, cobalt, iron, copper, or zinc complexes of the above mentioned dyes, and mixtures thereof.

The strong absorbing dye blocks off visible light in the wavelength range of from about 400 nm to about 515 nm, the most sensitive region of light known to induce light shock. The protective outer layer can be applied and removed with a relatively non-toxic solvent such as isopropanol, ethanol, butylacetate, alcohol ester, D-limonene, propylene glycol or the like. Additionally, due to the low strength of the resin, the protective outer layer also does not last for many copies in print engines and thus will be entirely removed after the initial cycles.

In embodiments, the protective outer layer or film is formed from a solution comprising the thermal plastic resin, yellow dye and film-forming binder dissolved in a solvent. In specific embodiments, the thermal plastic, film-forming resin is present in an amount of from about 1 percent to about 80 percent, or from about 2 percent to about 60 percent, or from

about 4 percent to about 30 percent by weight of the total weight of the protective outer layer solution. In specific embodiments, the yellow dye is present in an amount of from about 0.1 percent to about 20 percent, or from about 0.5 percent to about 10 percent, or from about 1 percent to about 5 percent by weight of the total weight of the protective outer layer solution. In further embodiments, the solvent is present in an amount of from about 10 percent to about 99 percent, or from about 20 percent to about 80 percent, or from about 30 percent to about 70 percent by weight of the total weight of the protective outer layer solution.

In embodiments, the thermal plastic resin is present in an amount of from about 5 percent to about 99 percent, or from about 30 percent to about 99 percent, or from about 40 percent to about 80 percent by weight of the total weight of the protective outer layer. In embodiments, the yellow dye is present in an amount of from about 1 percent to about 80 percent, or from about 5 percent to about 60 percent, or from about 10 percent to about 40 percent by weight of the total weight of the protective outer layer.

In the present embodiments, the protective outer layer has a thickness of from about 100 nm to about 10,000 nm, or a thickness of from about 200 nm to about 5,000 nm, or a thickness of from about 500 nm to about 2,000 nm.

In embodiments the protective outer layer or film can be manually applied, similar to the way in which powder lubricant, like KYNAR, is dusted onto drum photoreceptors during cartridge manufacturing, so that there will be no substantially added cost.

#### The Substrate

The photoreceptor support substrate **10** may be opaque or substantially transparent, and may comprise any suitable organic or inorganic material having the requisite mechanical properties. The entire substrate can comprise the same material as that in the electrically conductive surface, or the electrically conductive surface can be merely a coating on the substrate. Any suitable electrically conductive material can be employed, such as for example, metal or metal alloy. Electrically conductive materials include copper, brass, nickel, zinc, chromium, stainless steel, conductive plastics and rubbers, aluminum, semitransparent aluminum, steel, cadmium, silver, gold, zirconium, niobium, tantalum, vanadium, hafnium, titanium, nickel, niobium, stainless steel, chromium, tungsten, molybdenum, paper rendered conductive by the inclusion of a suitable material therein or through conditioning in a humid atmosphere to ensure the presence of sufficient water content to render the material conductive, indium, tin, metal oxides, including tin oxide and indium tin oxide, and the like. It could be single metallic compound or dual layers of different metals and/or oxides.

The substrate **10** can also be formulated entirely of an electrically conductive material, or it can be an insulating material including inorganic or organic polymeric materials, such as MYLAR, a commercially available biaxially oriented polyethylene terephthalate from DuPont, or polyethylene naphthalate available as KALEDEX 2000, with a ground plane layer **12** comprising a conductive titanium or titanium/zirconium coating, otherwise a layer of an organic or inorganic material having a semiconductive surface layer, such as indium tin oxide, aluminum, titanium, and the like, or exclusively be made up of a conductive material such as, aluminum, chromium, nickel, brass, other metals and the like. The thickness of the support substrate depends on numerous factors, including mechanical performance and economic considerations.

The substrate **10** may have a number of many different configurations, such as for example, a plate, a cylinder, a

drum, a scroll, an endless flexible belt, and the like. In the case of the substrate being in the form of a belt, as shown in FIG. 2, the belt can be seamed or seamless. In embodiments, the photoreceptor herein is in a drum configuration as shown in FIG. 1.

The thickness of the substrate **10** depends on numerous factors, including flexibility, mechanical performance, and economic considerations. The thickness of the support substrate **10** of the present embodiments may be at least about 500 micrometers, or no more than about 3,000 micrometers, or be at least about 750 micrometers, or no more than about 2500 micrometers.

An exemplary substrate support **10** is not soluble in any of the solvents used in each coating layer solution, is optically transparent or semi-transparent, and is thermally stable up to a high temperature of about 150° C. A substrate support **10** used for imaging member fabrication may have a thermal contraction coefficient ranging from about  $1 \times 10^{-5}$  per °C. to about  $3 \times 10^{-5}$  per °C. and a Young's Modulus of between about  $5 \times 10^{-5}$  psi ( $3.5 \times 10^{-4}$  Kg/cm<sup>2</sup>) and about  $7 \times 10^{-5}$  psi ( $4.9 \times 10^{-4}$  Kg/cm<sup>2</sup>).

#### The Ground Plane

The electrically conductive ground plane **12** may be an electrically conductive metal layer which may be formed, for example, on the substrate **10** by any suitable coating technique, such as a vacuum depositing technique. Metals include aluminum, zirconium, niobium, tantalum, vanadium, hafnium, titanium, nickel, stainless steel, chromium, tungsten, molybdenum, and other conductive substances, and mixtures thereof. The conductive layer may vary in thickness over substantially wide ranges depending on the optical transparency and flexibility desired for the electrophotoconductive member. Accordingly, for a flexible photoresponsive imaging device, the thickness of the conductive layer may be at least about 20 Angstroms, or no more than about 750 Angstroms, or at least about 50 Angstroms, or no more than about 200 Angstroms for an optimum combination of electrical conductivity, flexibility and light transmission.

Regardless of the technique employed to form the metal layer, a thin layer of metal oxide forms on the outer surface of most metals upon exposure to air. Thus, when other layers overlying the metal layer are characterized as "contiguous" layers, it is intended that these overlying contiguous layers may, in fact, contact a thin metal oxide layer that has formed on the outer surface of the oxidizable metal layer. Generally, for rear erase exposure, a conductive layer light transparency of at least about 15 percent is desirable. The conductive layer need not be limited to metals. Other examples of conductive layers may be combinations of materials such as conductive indium tin oxide as transparent layer for light having a wavelength between about 4000 Angstroms and about 9000 Angstroms or a conductive carbon black dispersed in a polymeric binder as an opaque conductive layer.

#### The Hole Blocking Layer

After deposition of the electrically conductive ground plane layer, the undercoat or hole blocking layer **14** may be applied thereto. Electron blocking layers for positively charged photoreceptors allow holes from the imaging surface of the photoreceptor to migrate toward the conductive layer. For negatively charged photoreceptors, any suitable hole blocking layer capable of forming a barrier to prevent hole injection from the conductive layer to the opposite photoconductive layer may be utilized. The hole blocking layer may include polymers such as polyvinylbutyral, epoxy resins, polyesters, polysiloxanes, polyamides, polyurethanes and the like, or may be nitrogen containing siloxanes or nitrogen containing titanium compounds such as trimethoxysilyl pro-

pylene diamine, hydrolyzed trimethoxysilyl propyl ethylene diamine, N-beta-(aminoethyl) gamma-amino-propyl trimethoxy silane, isopropyl 4-aminobenzene sulfonyl, di(dodecylbenzene sulfonyl)titanate, isopropyl di(4-aminobenzoyl)isostearoyl titanate, isopropyl tri(N-ethylaminoethylamino)titanate, isopropyl trianthranil titanate, isopropyl tri(N,N-dimethylaminolamino)titanate, titanium-4-amino benzene sulfonate oxyacetate, titanium 4-aminobenzoate isostearate oxyacetate,  $[H_2N(CH_2)_4]CH_3Si(OCH_3)_2$ , (gamma-aminobutyl)methyl diethoxysilane, and  $[H_2N(CH_2)_3]CH_3Si(OCH_3)_2$  (gamma-aminopropyl)methyl diethoxysilane, as disclosed in U.S. Pat. Nos. 4,338,387, 4,286,033 and 4,291,110.

General embodiments of the undercoat layer may comprise a metal oxide and a resin binder. The metal oxides that can be used with the embodiments herein include, but are not limited to, titanium oxide, zinc oxide, tin oxide, aluminum oxide, silicon oxide, zirconium oxide, indium oxide, molybdenum oxide, and mixtures thereof. Undercoat layer binder materials may include, for example, polyesters, MOR-ESTER 49,000 from Morton International Inc., VITEL PE-100, VITEL PE-200, VITEL PE-200D, and VITEL PE-222 from Goodyear Tire and Rubber Co., polyarylates such as ARDEL from AMOCO Production Products, polysulfone from AMOCO Production Products, polyurethanes, and the like.

The hole blocking layer should be continuous and have a thickness of less than about 0.5 micrometer because greater thicknesses may lead to undesirably high residual potential. A hole blocking layer of between about 0.005 micrometer and about 0.3 micrometer is used because charge neutralization after the exposure step is facilitated and optimum electrical performance is achieved. A thickness of between about 0.03 micrometer and about 0.06 micrometer is used for hole blocking layers for optimum electrical behavior. The blocking layer may be applied by any suitable conventional technique such as spraying, dip coating, draw bar coating, gravure coating, silk screening, air knife coating, reverse roll coating, vacuum deposition, chemical treatment and the like. For convenience in obtaining thin layers, the blocking layer is applied in the form of a dilute solution, with the solvent being removed after deposition of the coating by conventional techniques such as by vacuum, heating and the like. Generally, a weight ratio of hole blocking layer material and solvent of between about 0.05:100 to about 0.5:100 is satisfactory for spray coating.

#### The Charge Generation Layer

The charge generation layer **18** may thereafter be applied to the undercoat layer **14**. Any suitable charge generation binder including a charge generating/photoconductive material, which may be in the form of particles and dispersed in a film forming binder, such as an inactive resin, may be utilized. Examples of charge generating materials include, for example, inorganic photoconductive materials such as amorphous selenium, trigonal selenium, and selenium alloys selected from the group consisting of selenium-tellurium, selenium-tellurium-arsenic, selenium arsenide and mixtures thereof, and organic photoconductive materials including various phthalocyanine pigments such as the X-form of metal free phthalocyanine, metal phthalocyanines such as vanadyl phthalocyanine and copper phthalocyanine, hydroxy gallium phthalocyanines, chlorogallium phthalocyanines, titanyl phthalocyanines, quinacridones, dibromo anthranthrone pigments, benzimidazole perylene, substituted 2,4-diamino-triazines, polynuclear aromatic quinones, enzimidazole perylene, and the like, and mixtures thereof, dispersed in a film forming polymeric binder. Selenium, selenium alloy, benzimidazole perylene, and the like and mixtures thereof

may be formed as a continuous, homogeneous charge generation layer. Benzimidazole perylene compositions are well known and described, for example, in U.S. Pat. No. 4,587,189, the entire disclosure thereof being incorporated herein by reference. Multi-charge generation layer compositions may be used where a photoconductive layer enhances or reduces the properties of the charge generation layer. Other suitable charge generating materials known in the art may also be utilized, if desired. The charge generating materials selected should be sensitive to activating radiation having a wavelength between about 400 and about 900 nm during the imagewise radiation exposure step in an electrophotographic imaging process to form an electrostatic latent image. For example, hydroxygallium phthalocyanine absorbs light of a wavelength of from about 370 to about 950 nanometers, as disclosed, for example, in U.S. Pat. No. 5,756,245.

Any suitable inactive resin materials may be employed as a binder in the charge generation layer **18**, including those described, for example, in U.S. Pat. No. 3,121,006, the entire disclosure thereof being incorporated herein by reference. Organic resinous binders include thermoplastic and thermosetting resins such as one or more of polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl butyral, polyvinyl acetate, polysiloxanes, polyacrylates, polyvinyl acetals, polyamides, polyimides, amino resins, phenylene oxide resins, terephthalic acid resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrene-butadiene copolymers, vinylidenechloride/vinylchloride copolymers, vinylacetate/vinylidene chloride copolymers, styrene-alkyd resins, and the like. Another film-forming polymer binder is PCZ-400 (poly(4,4'-dihydroxy-diphenyl-1-1-cyclohexane) which has a viscosity-molecular weight of 40,000 and is available from Mitsubishi Gas Chemical Corporation (Tokyo, Japan).

The charge generating material can be present in the resinous binder composition in various amounts. Generally, at least about 5 percent by volume, or no more than about 90 percent by volume of the charge generating material is dispersed in at least about 95 percent by volume, or no more than about 10 percent by volume of the resinous binder, and more specifically at least about 20 percent, or no more than about 60 percent by volume of the charge generating material is dispersed in at least about 80 percent by volume, or no more than about 40 percent by volume of the resinous binder composition.

In specific embodiments, the charge generation layer **18** may have a thickness of at least about 0.1  $\mu\text{m}$ , or no more than about 2  $\mu\text{m}$ , or of at least about 0.2  $\mu\text{m}$ , or no more than about 1  $\mu\text{m}$ . These embodiments may be comprised of chlorogallium phthalocyanine or hydroxygallium phthalocyanine or mixtures thereof. The charge generation layer **18** containing the charge generating material and the resinous binder material generally ranges in thickness of at least about 0.1  $\mu\text{m}$ , or no more than about 5  $\mu\text{m}$ , for example, from about 0.2  $\mu\text{m}$  to about 3  $\mu\text{m}$  when dry. The charge generation layer thickness is generally related to binder content. Higher binder content compositions generally employ thicker layers for charge generation.

#### The Charge Transport Layer

In a drum photoreceptor, the charge transport layer comprises a single layer of the same composition. As such, the charge transport layer will be discussed specifically in terms

of a single layer **20**, but the details will be also applicable to an embodiment having dual charge transport layers. The charge transport layer **20** is thereafter applied over the charge generation layer **18** and may include any suitable transparent organic polymer or non-polymeric material capable of supporting the injection of photogenerated holes or electrons from the charge generation layer **18** and capable of allowing the transport of these holes/electrons through the charge transport layer to selectively discharge the surface charge on the imaging member surface. In one embodiment, the charge transport layer **20** not only serves to transport holes, but also protects the charge generation layer **18** from abrasion or chemical attack and may therefore extend the service life of the imaging member. The charge transport layer **20** can be a substantially non-photoconductive material, but one which supports the injection of photogenerated holes from the charge generation layer **18**.

The layer **20** is normally transparent in a wavelength region in which the electrophotographic imaging member is to be used when exposure is affected there to ensure that most of the incident radiation is utilized by the underlying charge generation layer **18**. The charge transport layer should exhibit excellent optical transparency with negligible light absorption and no charge generation when exposed to a wavelength of light useful in xerography, e.g., 400 to 900 nanometers. In the case when the photoreceptor is prepared with the use of a transparent substrate **10** and also a transparent or partially transparent conductive layer **12**, image wise exposure or erase may be accomplished through the substrate **10** with all light passing through the back side of the substrate. In this case, the materials of the layer **20** need not transmit light in the wavelength region of use if the charge generation layer **18** is sandwiched between the substrate and the charge transport layer **20**. The charge transport layer **20** in conjunction with the charge generation layer **18** is an insulator to the extent that an electrostatic charge placed on the charge transport layer is not conducted in the absence of illumination. The charge transport layer **20** should trap minimal charges as the charge passes through it during the discharging process.

The charge transport layer **20** may include any suitable charge transport component or activating compound useful as an additive dissolved or molecularly dispersed in an electrically inactive polymeric material, such as a polycarbonate binder, to form a solid solution and thereby making this material electrically active. "Dissolved" refers, for example, to forming a solution in which the small molecule is dissolved in the polymer to form a homogeneous phase; and molecularly dispersed in embodiments refers, for example, to charge transporting molecules dispersed in the polymer, the small molecules being dispersed in the polymer on a molecular scale. The charge transport component may be added to a film forming polymeric material which is otherwise incapable of supporting the injection of photogenerated holes from the charge generation material and incapable of allowing the transport of these holes through. This addition converts the electrically inactive polymeric material to a material capable of supporting the injection of photogenerated holes from the charge generation layer **18** and capable of allowing the transport of these holes through the charge transport layer **20** in order to discharge the surface charge on the charge transport layer. The high mobility charge transport component may comprise small molecules of an organic compound which cooperate to transport charge between molecules and ultimately to the surface of the charge transport layer. For example, but not limited to, N,N'-diphenyl-N,N'-bis(3-methyl phenyl)-1,1'-biphenyl-4,4'-diamine (TPD), other arylamines

## 11

like triphenyl amine, N,N,N',N'-tetra-p-tolyl-1,1'-biphenyl-4,4'-diamine (TM-TPD), and the like.

A number of charge transport compounds can be included in the charge transport layer, which layer generally is of a thickness of from about 5 to about 75 micrometers, and more specifically, of a thickness of from about 15 to about 40 micrometers. Examples of charge transport components are aryl amines of the following formulas/structures:



wherein X is a suitable hydrocarbon like alkyl, alkoxy, aryl, and derivatives thereof; a halogen, or mixtures thereof, and especially those substituents selected from the group consisting of Cl and CH<sub>3</sub>; and molecules of the following formulas



wherein X, Y and Z are independently alkyl, alkoxy, aryl, a halogen, or mixtures thereof, and wherein at least one of Y and Z are present.

Alkyl and alkoxy contain, for example, from 1 to about 25 carbon atoms, and more specifically, from 1 to about 12 carbon atoms, such as methyl, ethyl, propyl, butyl, pentyl, and the corresponding alkoxides. Aryl can contain from 6 to about 36 carbon atoms, such as phenyl, and the like. Halogen includes chloride, bromide, iodide, and fluoride. Substituted alkyls, alkoxy, and aryls can also be selected in embodiments.

Examples of specific aryl amines that can be selected for the charge transport layer include N,N'-diphenyl-N,N'-bis(alkylphenyl)-1,1'-biphenyl-4,4'-diamine wherein alkyl is selected from the group consisting of methyl, ethyl, propyl, butyl, hexyl, and the like; N,N'-diphenyl-N,N'-bis(halophenyl)-1,1'-biphenyl-4,4'-diamine wherein the halo substituent is a chloro substituent; N,N'-bis(4-butylphenyl)-N,N'-di-p-tolyl-[p-terphenyl]-4,4'-diamine, N,N'-bis(4-butylphenyl)-N,N'-di-m-tolyl-[p-terphenyl]-4,4'-diamine, N,N'-bis(4-butylphenyl)-N,N'-di-o-tolyl-[p-terphenyl]-4,4'-diamine, N,N'-bis(4-butylphenyl)-N,N'-bis(4-isopropylphenyl)-[p-terphenyl]-4,4'-diamine, N,N'-bis(4-butylphenyl)-N,N'-bis(2-ethyl-6-methylphenyl)-[p-terphenyl]-4,4'-diamine, N,N'-bis(4-butylphenyl)-N,N'-bis(2,5-dimethylphenyl)-[p-terphenyl]-4,4'-diamine, N,N'-diphenyl-N,N'-bis(3-chlorophenyl)-[p-terphenyl]-4,4'-diamine, and the like. Other known charge transport layer molecules may be selected in embodiments, reference for example, U.S. Pat. Nos. 4,921,773 and 4,464,450, the disclosures of which are totally incorporated herein by reference.

Examples of the binder materials selected for the charge transport layers include components, such as those described in U.S. Pat. No. 3,121,006, the disclosure of which is totally incorporated herein by reference. Specific examples of polymer binder materials include polycarbonates, polyarylates, acrylate polymers, vinyl polymers, cellulose polymers, polyesters, polysiloxanes, polyamides, polyurethanes, poly(cycloolefins), and epoxies, and random or alternating copolymers thereof. In embodiments, the charge transport layer, such as a hole transport layer, may have a thickness of at least about 10 μm, or no more than about 40 μm.

Examples of components or materials optionally incorporated into the charge transport layers or at least one charge transport layer to, for example, enable improved lateral charge migration (LCM) resistance include hindered phenolic antioxidants such as tetrakis methylene(3,5-di-tert-butyl-4-hydroxy hydrocinnamate) methane (IRGANOX® 1010, available from Ciba Specialty Chemical), butylated hydroxytoluene (BHT), and other hindered phenolic antioxidants including SUMILIZER™ BHT-R, MDP-S, BBM-S, WX-R, NW, BP-76, BP-101, GA-80, GM and GS (available from Sumitomo Chemical Co., Ltd.), IRGANOX® 1035, 1076, 1098, 1135, 1141, 1222, 1330, 1425WL, 1520L, 245, 259, 3114, 3790, 5057 and 565 (available from Ciba Specialties Chemicals), and ADEKA STAB™ AO-20, AO-30, AO-40, AO-50, AO-60, AO-70, AO-80 and AO-330 (available from Asahi Denka Co., Ltd.); hindered amine antioxidants such as SANOL™ LS-2626, LS-765, LS-770 and LS-744 (available from SANKYO CO., Ltd.), TINUVIN® 144 and 622LD (available from Ciba Specialties Chemicals), MARK™ LA57, LA67, LA62, LA68 and LA63 (available from Asahi Denka Co., Ltd.), and SUMILIZER® TPS (available from Sumitomo Chemical Co., Ltd.); thioether antioxidants such as SUMILIZER® TP-D (available from Sumitomo Chemical Co., Ltd.); phosphite antioxidants such as MARK™ 2112, PEP-8, PEP-24G, PEP-36, 329K and HP-10 (available from Asahi Denka Co., Ltd.); other molecules such as bis(4-diethylamino-2-methylphenyl)phenylmethane (BDETPM), bis-[2-methyl-4-(N-2-hydroxyethyl-N-ethylaminophenyl)]-phenylmethane (DHTPM), and the like. The weight percent of the antioxidant in at least one of the charge transport layer is from about 0 to about 20, from about 1 to about 10, or from about 3 to about 8 weight percent.

The charge transport layer should be an insulator to the extent that the electrostatic charge placed on the hole transport layer is not conducted in the absence of illumination at a rate sufficient to prevent formation and retention of an electrostatic latent image thereon. The charge transport layer is substantially nonabsorbing to visible light or radiation in the region of intended use, but is electrically "active" in that it allows the injection of photogenerated holes from the photoconductive layer, that is the charge generation layer, and allows these holes to be transported through itself to selectively discharge a surface charge on the surface of the active layer.

## 12

## 13

In addition, in the present embodiments using a belt configuration, the charge transport layer may consist of a single pass charge transport layer or a dual pass charge transport layer (or dual layer charge transport layer) with the same or different transport molecule ratios. In these embodiments, the dual layer charge transport layer has a total thickness of from about 10  $\mu\text{m}$  to about 40  $\mu\text{m}$ . In other embodiments, each layer of the dual layer charge transport layer may have an individual thickness of from 2  $\mu\text{m}$  to about 20  $\mu\text{m}$ . Moreover, the charge transport layer may be configured such that it is used as a top layer of the photoreceptor to inhibit crystallization at the interface of the charge transport layer and the overcoat layer. In another embodiment, the charge transport layer may be configured such that it is used as a first pass charge transport layer to inhibit microcrystallization occurring at the interface between the first pass and second pass layers.

Any suitable and conventional technique may be utilized to form and thereafter apply the charge transport layer mixture to the supporting substrate layer. The charge transport layer may be formed in a single coating step or in multiple coating steps. Dip coating, ring coating, spray, gravure or any other drum coating methods may be used.

Drying of the deposited coating may be effected by any suitable conventional technique such as oven drying, infra red radiation drying, air drying and the like. The thickness of the charge transport layer after drying is from about 10  $\mu\text{m}$  to about 40  $\mu\text{m}$  or from about 12  $\mu\text{m}$  to about 36  $\mu\text{m}$  for optimum photoelectrical and mechanical results. In another embodiment the thickness is from about 14  $\mu\text{m}$  to about 36  $\mu\text{m}$ .

## The Overcoat Layer

Other layers of the imaging member may include, for example, an optional over coat layer 32. An optional overcoat layer 32, if desired, may be disposed over the charge transport layer 20 to provide imaging member surface protection as well as improve resistance to abrasion. In embodiments, the overcoat layer 32 may have a thickness ranging from about 0.1 micrometer to about 10 micrometers or from about 1 micrometer to about 10 micrometers, or in a specific embodiment, about 3 micrometers.

These overcoating layers may include thermoplastic organic polymers or inorganic polymers that are electrically insulating or slightly semi-conductive. For example, overcoat layers may be fabricated from a dispersion including a particulate additive in a resin. Suitable particulate additives for overcoat layers include metal oxides including aluminum oxide, non-metal oxides including silica or low surface energy polytetrafluoroethylene (PTFE), and combinations thereof. Suitable resins include those described above as suitable for photogenerating layers and/or charge transport layers, for example, polyvinyl acetates, polyvinylbutyral, polyvinylchlorides, vinylchloride and vinyl acetate copolymers, carboxyl-modified vinyl chloride/vinyl acetate copolymers, hydroxyl-modified vinyl chloride/vinyl acetate copolymers, carboxyl- and hydroxyl-modified vinyl chloride/vinyl acetate copolymers, polyvinyl alcohols, polycarbonates, polyesters, polyurethanes, polystyrenes, polybutadienes, polysulfones, polyarylethers, polyarylsulfones, polyethersulfones, polyethylenes, polypropylenes, polymethylpentenes, polyphenylene sulfides, polysiloxanes, polyacrylates, polyvinyl acetals, polyamides, polyimides, amino resins, phenylene oxide resins, terephthalic acid resins, phenoxy resins, epoxy resins, phenolic resins, polystyrene and acrylonitrile copolymers, poly-N-vinylpyrrolidinones, acrylate copolymers, alkyd resins, cellulosic film formers, poly(amideimide), styrene-butadiene copolymers, vinylidenechloride-vinylchloride copolymers, vinylacetate-vinylidenechloride copolymers, styrene-alkyd resins, polyvinylcarbazoles, and combinations thereof.

## 14

ride copolymers, vinylacetate-vinylidenechloride copolymers, styrene-alkyd resins, polyvinylcarbazoles, and combinations thereof.

In embodiments, the overcoat layer is formed from a formulation or solution comprising a small transport molecule, a resin, a crosslinker compound, an acid catalyst, and one or more surface additives in a solvent. To facilitate the crosslinking process, the combination of the small transport molecule and the crosslinker compound takes place in the presence of a strong acid solution.

In embodiments the small transport molecule can be selected from the group consisting of N,N'-bis[4-n-butylphenyl]-N,N'-di[3-hydroxyphenyl]-terphenyl-diamine (DHTER), N,N'-diphenyl-N,N'-bis(3-hydroxyphenyl)-[1,1'-biphenyl]-4,4'-diamine (DHTBD), and the like, and mixtures thereof. In embodiments, the resin can be a polyol, and the like. One specific resin used is JONCRYL, an acrylic polyol, available from BASF Corp. (Florham Park, N.J.). The crosslinker compound may be, in embodiments, a melamine formaldehyde compound, and the like. In one example, the melamine formaldehyde crosslinker compound is CYMEL 303, available from Cytec Corporation (West Paterson, N.J.). An acid catalyst may be toluenesulfonic acid, and the like. In embodiments, the acid catalyst used is NACURE XP-357 available from King Industries (Norwalk, Conn.). In specific embodiments, the surface additive is SILCLEAN 3700, a solution of a silicone modified polyacrylate (OH-functional) which can be crosslinked into a polymer network due to its —OH functionality. SILCLEAN 3700 is available from BYK-Chemie GmbH (Wesel, Germany). The solvent may be an alcohol and the like. In one embodiment, the solvent used is a glycol ether and is available at about 20 percent solids (DOWANOL PM), available from The Dow Chemical Co. (Midland, Mich.).

Overcoating layers may be continuous and have a thickness of at least about 0.5 micrometer, or no more than 10 micrometers, and in further embodiments have a thickness of at least about 2 micrometers, or no more than 6 micrometers.

Various exemplary embodiments encompassed herein include a method of imaging which includes generating an electrostatic latent image on an imaging member, developing a latent image, and transferring the developed electrostatic image to a suitable substrate.

While the description above refers to particular embodiments, it will be understood that many modifications may be made without departing from the spirit thereof. The accompanying claims are intended to cover such modifications as would fall within the true scope and spirit of embodiments herein.

The presently disclosed embodiments are, therefore, to be considered in all respects as illustrative and not restrictive, the scope of embodiments being indicated by the appended claims rather than the foregoing description. All changes that come within the meaning of and range of equivalency of the claims are intended to be embraced therein.

## EXAMPLES

The example set forth herein below and is illustrative of different compositions and conditions that can be used in practicing the present embodiments. All proportions are by weight unless otherwise indicated. It will be apparent, however, that the embodiments can be practiced with many types of compositions and can have many different uses in accordance with the disclosure above and as pointed out hereinafter.

To understand the underlying causes, the light shock effect on PASCO was investigated by preparing lab devices using two PASCO formulations (PASCO 4 and PASCO 5) as well as varying charge generation layer thickness and heating time. The PASCO 4 formulation is consisted of 34 parts in weight of N,N'-diphenyl-N,N'-bis(3-hydroxyphenyl)-[1,1'-biphenyl]-4,4'-diamine (DHTBD), 26 parts of JONCRYL 585, an acrylic polyol, available from BASF Corp. (Florham Park, N.J.), 37 parts of CYMEL 303, a melamine formaldehyde compound available from Cytec Corporation (West Paterson, N.J.), 1.1 parts of NACURE XP-357, an acid catalyst available from King Industries (Norwalk, Conn.), 1.3 parts of SILCLEAN 3700, a solution of a silicone modified polyacrylate (OH-functional) available from BYK-Chemie GmbH (Wesel, Germany). The above ingredients are dissolved at about 22% in solids in a solvent of Dowanol PM available from The Dow Chemical Co. (Midland, Mich.). The PASCO 5 formulation is consisted of 55.6 parts in weight of N,N'-diphenyl-N,N'-bis(3-hydroxyphenyl)-[1,1'-biphenyl]-4,4'-diamine (DHTBD), 42 parts of CYMEL 303, a melamine formaldehyde compound available from Cytec Corporation (West Paterson, N.J.), 1.2 parts of NACURE XP-357, an acid catalyst available from King Industries (Norwalk, Conn.), 1.4 parts of SILCLEAN 3700, a solution of a silicone modified polyacrylate (OH-functional) available from BYK-Chemie GmbH (Wesel, Germany). The PASCO 5 formulation does not contain a polyol. The above ingredients are dissolved at about 22% in solids in a solvent of Dowanol PM available from The Dow Chemical Co. (Midland, Mich.).

Reference devices were also prepared with a regular charge transport layer of 26  $\mu\text{m}$  in thickness with regular or thick charge generation layers, where the charge generation layer solution was at a solid content of 5.8% in weight regular charge generation layer was prepared at a dip coating pull rate of 130 mm/minute and the thick charge generation layer was prepared at a dip coating pull rate of 250 mm/minute, and with regular heating or extra heating, where the extra heating was an additional heating of 155  $^{\circ}\text{C}$  at 30 minutes under the PASCO curing conditions. Table 1 shows the light shock test results from the comparative experiment.

TABLE 1

| Charge Generation Pull Rate | Extra Heating | OC Type | $\Delta V_{low}$ |
|-----------------------------|---------------|---------|------------------|
| 250                         | NO            | NO      | 20               |
| 250                         | YES           | NO      | 39               |
| 250                         | YES           | PASCO 4 | 136              |
| 250                         | YES           | PASCO 5 | 118              |
| 130                         | NO            | NO      | 24               |
| 130                         | YES           | NO      | 34               |
| 130                         | YES           | PASCO 4 | 142              |
| 130                         | YES           | PASCO 5 | 37               |

For the regular charge transport layer, the extra heating contributed to about 10-20 V more in light shock and only about 5 V increase with the thicker charge generation layer. For PASCO 4, it appears that, at least for this set of experimental devices, charge generation layer thickness did not have much effect on light shock as both devices exhibited a substantial change in surface potential. In contrast, PASCO 5 appears to have only a small light shock voltage at regular charge generation layer thickness but the  $\Delta V_{low}$  increased significantly with thick charge generation layer. Marginal means plots of  $\Delta V_{low}$  ( $1.5 \text{ ergs/cm}^2$ ) are shown in FIG. 3.

Experiments initially began by focusing on several UV-blocking dyes such as 2-2'-dihydroxy-4-methylbenzophenone (such as CYASORB UV-24 available from Cytec Industries Inc. (Woodland Park, N.J.)) and ethyl-2-cyano-3,3-diphenylacrylate (such as UVINUL 3035 available from BASF Corp. (Florham Park, N.J.)).

The UV absorption layer was formulated with about 20 wt. percent to about 30 wt. percent of conventional poly-vinyl butyral binder (such as B98 available from Monsanto Chemical (St. Louis, Mo.)) in isopropanol or like solvent. B98 may be used as the binder to allow good film forming properties. Typically, a solution of about 2 wt percent of the binder was used and the protective layer solution was applied by wiping the PASCO photoreceptor surface with a paper towel or using laboratory dip coating equipment, such as for example, a Tsukiage coater. The UV dyes were found to have no, or at most, minuscule improvement on light shock.

Thus, subsequent yellow dyes were pursued, in conjunction with an optional UV light blocker, to further investigate the effect of light blockage. FIG. 4 shows film UV-Vis spectra of several UV and yellow dyes and PASCO 4 and PASCO 5 that were investigated. All spectra were normalized to their peak values. It is evident that, by using some yellow dyes having high optical strength, the visible light from 400-515 nm can be effectively blocked.

As shown in FIG. 4, the yellow dyes, particularly a metal-free monoazo dye (such as CIBA ORASOL YELLOW 4GN available from Ciba Specialty Chemicals) was found to be most effective in reducing light shock for the tested devices. ORASOL YELLOW 2GLN is a metal-free azo dye and BASANTOL YELLOW 215 is an azo cobalt complex. With about 1  $\mu\text{m}$  of the protective outer layer, the effective thickness was only about 200 nm for a protective outer layer comprising 20 wt percent dye and 80 wt percent PVB binder. This formulation reduced both  $\Delta V_{(1.86)}$  and  $\Delta V_{er}$  to only about 45 V, in contrast to 146 V and 100 V, respectively for the PASCO control area.

For further comparison, regular non-overcoated photoreceptor drums with regular charge generation thickness have about 20 V in light shock. Replacing some of the yellow dye with UV-24 dye or green food colorant, which contains unknown amounts of a yellow and blue dyes, did not seem to help the light shock. FIG. 5 shows light shock test results for various dye samples (dye-only) and their controls (areas not coated with protection outer layer solution).

A repeat experiment for the metal-free monoazo was executed on PASCO steady state drums. Again, that specific dye was found to be most effective in reducing light shock for the tested PASCO devices. With about 1.2  $\mu\text{m}$  of the protective outer layer, the effective thickness was about 250 nm for a protective outer layer comprising 20 wt percent dye and 80 wt percent PVB binder. This formulation reduced both  $\Delta V_{(1.86)}$  and  $\Delta V_{er}$  to only about 15-20 V, in contrast to 103 V and 62 V, respectively for the control area on the same device. Table 2 summarizes light shock test results for the experiment.

TABLE 1

|                              | $\Delta V_{(1.5)}$ | $\Delta V_{er}$ |
|------------------------------|--------------------|-----------------|
| 1 $\mu\text{m}$ Yellow 4GN   | 19                 | 16              |
| Control                      | 103                | 62              |
| 0.2 $\mu\text{m}$ Yellow 4GN | 74                 | 52              |
| Control                      | 116                | 72              |

The PASCO device containing a 0.2  $\mu\text{m}$  yellow dye layer was print tested in a xerographic engine and time=0 results

showed nominal prints, similar to regular devices. Separately, the 1  $\mu\text{m}$  protective outer layer device was wiped with isopropanol and the layer was easily removed with no visible presence of the protective outer layer left.

To verify that the protective outer layer is readily removed in print engines when under operation, a 30 mm drum imaging member was coated with a similar 1  $\mu\text{m}$  protective outer layer and tested in a wear test fixture, where only charging and development were acting on the device without transfer. By stopping the wear fixture at run cycles of 50 or 100, the imaging member was taken out of the fixture and visibly inspected. It was found that between 100-150 cycles, the protective outer layer started showing substantial reduction in color density and between 300-500 cycles, the protective outer layer was completely gone, suggesting the protective outer layer can be indeed a good sacrificial layer for reducing light shock for PASCO devices.

All the patents and applications referred to herein are hereby specifically, and totally incorporated herein by reference in their entirety in the instant specification.

It will be appreciated that several of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

The invention claimed is:

1. A light shock resistant imaging member, comprising: a substrate;

a charge generation layer disposed on the substrate; 35 a charge transport layer disposed on the charge generation layer;

an overcoat layer disposed on the charge transport layer; and

a removable protective outer film disposed on the overcoat 40 layer, comprising:

a low-strength film-forming thermal plastic resin, and a yellow dye disposed throughout the thermal plastic

resin, wherein the removable protective outer film blocks ultraviolet or visible light in the range of from about 400 nm to about 515 nm from the imaging member and is removed from the imaging member with a solvent or a cleaning component within 500 cycles of operation of the imaging member.

2. The imaging member of claim 1, wherein the thermal plastic resin is selected from the group consisting of polyvinyl butyral, polyester, polycarbonate, polystyrene, melamine formaldehyde resins, polyacrylamide, polyurethane, polysulfonate, polyacrylonitrile, polyethylene glycol, poly(methyl acrylate), poly(methyl methacrylate), and mixtures thereof.

3. The imaging member of claim 1, wherein the yellow dye is selected from the group consisting of azo, metal-free monoazo dye, 2-2'-Dihydroxy-4-methoxybenzophene, oxybenzone, tartrazine, quinophthaleone, pyrazolone, methane, coumarin, and chromium, cobalt, iron, copper, or zinc complexes of the above mentioned dyes, and mixtures thereof.

4. The imaging member of claim 1, wherein the thermal plastic resin is present in the protective outer film in an amount of from about 10 percent to about 99 percent by total weight of the protective outer film.

5. The imaging member of claim 1, wherein the yellow dye is present in the protective outer film in an amount of from about 1 percent to about 90 percent by total weight of the protective outer film.

6. The imaging member of claim 1, wherein the protective outer film is removable by solvent.

7. The imaging member of claim 1, wherein the protective outer film is removed after from about 100 to about 500 cycles.

8. An image forming apparatus for forming images on a recording medium comprising:

a) a light shock resistant imaging member having a charge retentive-surface for receiving an electrostatic latent image thereon, wherein the imaging member comprises a substrate, a charge generation layer disposed on the substrate, a charge transport layer disposed on the charge generation layer, an overcoat layer disposed on the charge transport layer, and a removable protective outer film disposed on the overcoat layer, comprising a low-strength film-forming thermal plastic resin, and a yellow dye disposed throughout the thermal plastic resin, wherein the removable protective outer film blocks ultraviolet or visible light in the range of from about 400 nm to about 515 nm from the imaging member;

b) a development component for applying a developer material to the charge-retentive surface to develop the electrostatic latent image to form a developed image on the charge-retentive surface;

c) a transfer component for transferring the developed image from the charge-retentive surface to a copy substrate;

d) a fusing component for fusing the developed image to the copy substrate; and

e) a cleaning component for removing any developer material remaining on the charge-retentive surface, wherein the cleaning component removes the removable protective layer within 500 cycles of operation of the image forming apparatus and directs the removed developer material to a toner waste container.

9. The image forming apparatus of claim 8, wherein the thermal plastic resin is selected from the group consisting of poly-vinyl butyral, polyester, polycarbonate, polystyrene, melamine formaldehyde resins, polyacrylamide, polyurethane, polysulfonate, polyacrylonitrile, polyethylene glycol, poly(methyl acrylate), poly(methyl methacrylate), and mixtures thereof.

10. The image forming apparatus of claim 8, wherein the yellow dye is selected from the group consisting of azo, metal-free monoazo dye, 2-2'-Dihydroxy-4-methoxybenzophene, oxybenzone, tartrazine, quinophthaleone, pyrazolone, methane, coumarin, and chromium, cobalt, iron, copper, or zinc complexes of the above mentioned dyes, and mixtures thereof.

11. The image forming apparatus of claim 8, wherein the thermal plastic resin is present in the protective outer film in an amount of from about 10 percent to about 99 percent by total weight of the protective outer film.

12. The image forming apparatus of claim 8, wherein the yellow dye is present in the protective outer film in an amount of from about 1 percent to about 90 percent by total weight of the protective outer film.